

Aug. 30, 1960

G. T. SEABORG ET AL

2,951,018

ELECTRODEPOSITION OF NEPTUNIUM

Filed Oct. 29, 1945

FIG. 1.



FIG. 2.



witnesses:

*Mayer A. Baerin*  
*John A. McElroy*

Inventors:

*Glenn T. Seaborg*  
*Arthur C. Wahl*  
By *Robert A. Sander*  
*Attorney.*

2,951,018

## ELECTRODEPOSITION OF NEPTUNIUM

Glenn T. Seaborg, Chicago, Ill., and Arthur C. Wahl, Santa Fe, N. Mex., assignors to the United States of America as represented by the United States Atomic Energy Commission

Filed Oct. 29, 1945, Ser. No. 625,136

1 Claim. (Cl. 204—1.5)

This invention relates to a method of separating certain new elements from solutions. More particularly it pertains to a process involving the electrolytic deposition of neptunium from solutions thereof.

It is known that plutonium can be produced in small quantities by the bombardment of natural uranium with neutrons. The designation "plutonium" or "element 94" as used throughout the present description refers to the transuranic element having an atomic number of 94. The expression "94<sup>239</sup>" means the isotope of element 94 has an atomic weight or mass of 239. Similarly, the terms "element 93" or "Np" refer to the new element known as neptunium having an atomic number of 93.

Uranium is composed of three isotopes, namely, U<sup>234</sup>, U<sup>235</sup> and U<sup>238</sup>, the latter being present in excess of 99 percent of the whole. When U<sup>238</sup> is subjected to the action of slow or thermal neutrons, a fourth isotope, U<sup>239</sup>, is produced having a half-life of 23 minutes and undergoes beta decay to Np<sup>239</sup> which decays further by beta radiation with a half-life of 2.3 days to yield plutonium. In addition to the formation of the transuranic elements, neptunium and plutonium, there are simultaneously produced other elements of lower atomic weight known as fission fragments. These fission fragments are composed of two distinct element groups, i.e., a light and heavy element group. The light group contains elements having atomic numbers of between about 35 and 46 while the heavier group is composed of elements of atomic numbers varying between about 51 and 60. The elements of these groups as originally produced are considerably overmassed and undercharged, and hence are highly unstable. By beta radiation, however, they quickly transform themselves into isotopes of these various elements having longer half-lives. The resulting materials are commonly known as fission products. It is particularly desirable to separate the neptunium and plutonium from the radioactive fission fragments and fission products thereby removing from the mass, subjected to neutron bombardment, the radioactive materials and particularly the light elements such as the light metals having very short half-lives.

It is an object of this invention to provide a simple and efficient means of separating neptunium from solutions and particularly carrying out this separation in a quantitative manner.

It is a further object of this invention to accomplish this result by electrolytic means without the use of added reagents and without the necessity of evaporating the solution to dryness.

Another object of the present invention is to provide a simple, rapid, and efficient means for producing a thin film of neptunium.

Further objects will be apparent from the accompanying drawing and the description which follows.

Subsequent to the bombardment of uranium with neutrons to produce new elements as discussed above, the usual procedure is to dissolve the entire mass in a suit-

able acid, such as nitric acid. This solution contains uranium, neptunium, plutonium, and all of the other products resulting from the fission of U<sup>235</sup>.

In view of the relatively short half-life of neptunium, it is important that any method of separation of this element employed be a rapid one involving a minimum consumption of time.

In the study of radioactive substances such as neptunium, it is often of great importance to obtain a very thin uniform layer of the substance in question so that its radioactivity can be measured. If the layer is too thick there will be self-absorption phenomena that will seriously interfere with radioactivity measurements.

In accordance with the present invention it has been found that neptunium may be recovered by electrodeposition from solutions thereof. Nonaqueous solutions of neptunium such as, solutions of neptunium nitrate in absolute ethyl alcohol or other organic solvent capable of supplying a pair of electrons to neptunium to form a co-ordinate linkage such as, acetone, methyl ethyl ketone, hexone, methanol, n-propanol, ethyl ether, cellosolve, formamid, acetamid, acetic acid or other solvent containing the group >C=O, —N=, —S—, etc., may be used for this purpose.

The aqueous solutions from which neptunium is deposited may vary widely in their hydrogen ion concentration; however, in the majority of instances it is generally preferable to employ a pH of between about 5 and 7. Suitable buffers such as acetic acid—sodium acetate, carbon dioxide—sodium bicarbonate buffers, etc. may be used to establish the desired pH.

The process of the present invention may be carried out in any standard electrolytic apparatus. A suitable apparatus is shown in Fig. 1 wherein the electrolyte 1 is contained in a glass cylinder 2 having a silver bottom 3 connected to lead line 4 which is in turn connected to a negative source of potential. Anode 5 and cathode 3 consist of platinum or insoluble anode material and silver, respectively and are connected to a suitable source of direct current such as a battery. The connection is made through switches 6 and 7 and variable resistance 8. In order to measure the amount of current used a milliammeter 9 with a switch connection 10 for low and high scale readings, is placed in the line. In order to measure the voltage with a very small current loss a microammeter 11 is placed across the line and in series with two fixed high resistances 12 and 13. As actually used resistance 12 is 0.1 megohm and resistance 13 is 1.0 megohm.

When using the apparatus the electrolyte consists preferably of neptunium nitrate and lanthanum nitrate in absolute alcohol. The current is passed through the solution and the amperage is adjusted by means of the variable resistance 8.

It was found that when carrying out such an electrolysis the amperage rises continuously with time as shown in Fig. 2.

In effecting the process of the present invention a relatively wide voltage range may be utilized. For the majority of instances, however, voltage of between about 2 and 50 volts have been found adequate for nonaqueous electrolytes and for aqueous medium a somewhat lower voltage, e.g. 2 to about 10 volts, is suitable. Likewise, the current densities used may cover a comparatively wide range, however, for most purposes it has been found entirely satisfactory to use current densities of between about 0.001 and 0.6 ampere per square decimeter. The temperatures employed may, in general, vary from about 30° C. to about 90° C.

The process of the present invention may be further illustrated by reference to the following specific examples.

In all instances the percentages of neptunium plated out was determined in the manner referred to in Example 1.

*Example 1*

To a solution of 2 cubic centimeters of neptunium nitrate was added 2.5 mg. of La<sup>+3</sup> as nitrate. Thereafter sufficient ammonium hydroxide was added to cause substantially complete precipitation of the lanthanum. The precipitate thus obtained, which contained the neptunium was separated by centrifugation, washed with ammonium hydroxide, dissolved in nitric acid and the resulting solution evaporated to dryness. The product thus obtained was again dissolved in nitric acid, evaporated to dryness on a steam bath, and dissolved in absolute alcohol. The precipitate did not entirely dissolve and the solution was filtered and diluted to 25 cubic centimeters with absolute alcohol. The solution was centrifuged to remove the small amount of precipitate still remaining.

Two cubic centimeters of this solution of neptunium nitrate and lanthanum nitrate in absolute alcohol was electrolyzed in an apparatus similar to that illustrated in Fig. 1. The electrolysis was carried out for forty-five minutes at 50 volts. The current density varied over the time of electrolysis from 1.8 to 4.7 milliamperes per square decimeter as shown in the curve of Figure 2. The electrodeposited neptunium was washed with absolute alcohol. On the basis of determinations of beta radiation from aliquot portions of the initial neptunium solution and the electrolyte after the plating operation, using standard counter tube techniques, it was found that 100 percent of the neptunium in solution was deposited on the cathode probably in the form of an oxide.

*Example 2*

One cubic centimeter of the solution prepared as described in Example 1, was mixed with 1 cubic centimeter of a solution of lanthanum nitrate in absolute alcohol. The resulting solution was electrolyzed using the apparatus shown in Fig. 1. The electrolysis was carried out for thirty-five minutes at 17 volts and a current density of 3 to 5 milliamperes per square decimeter. Forty-eight percent of the neptunium was plated out. With 2 cubic centimeters of the electrolyte described in Example 1, 81 percent of the neptunium was plated out, using a voltage of between 20 and 40 volts and a current of 2-4 milliamperes per square decimeter for a period of fifteen minutes.

*Example 3*

A solution of a small quantity of neptunium prepared by dissolving neutron bombarded uranium in nitric acid in an acetate buffered aqueous medium having a pH of 5 and containing no carrier was subjected to electrolysis for two hours at a current density of 0.16 ampere per square decimeter and a potential of 8 volts, using a mercury cathode. Sixty-three percent of the neptunium was found in the mercury, 6.5 percent remained in the aqueous electrolyte, and 31.5 percent was unaccounted for. The latter was probably lost in the step in which the

last traces of lanthanum carrier were removed from the neptunium in the process of separating that element from the nitric acid solution of neutron bombarded uranium.

*Example 4*

10 A solution containing a small amount of neptunium in one molal ammonium acetate solution was electrolyzed for fifty minutes. The current density was 0.15 ampere per square decimeter, at a voltage of from 2.4 to 2.7. The temperature was maintained at from 79° to 84° C. Seventy-four percent of the neptunium was removed from this solution probably in the form of oxide.

*Example 5*

15 An aqueous molal ammonium acetate solution containing .01 mole of uranyl ion (UO<sub>2</sub><sup>++</sup>) and a tracer quality of neptunium was subjected to electrolysis at a current density of 0.15 ampere per square decimeter and at a voltage of from about 2.4 to 2.7 volts. The temperature 20 of the solution was maintained at from about 79° to 84° C. The electrolysis was carried out for about sixty-five minutes, at the end of which time 97 percent of the neptunium, probably as an oxide, and 98 percent of the 25 uranium had been removed from the solution.

25 It is to be strictly understood that the foregoing examples are merely illustrative and are in no way limitative. It will be apparent to those skilled in the art that the present invention is susceptible of numerous improvements and modifications without departing from the scope thereof. For example, the current density employed may be substantially higher than specified in the foregoing description merely by using a rotating cathode, increasing the rate of agitation, or altering the bath temperature. In general, it may be said that any procedure for the recovery of neptunium based upon the electrolytic deposition 30 thereof from its solution is to be regarded as lying within the scope of this invention.

What is claimed is:

35 The process of electrodepositing neptunium from solutions thereof, which comprises conducting the electrodeposition from an absolute alcohol bath containing a neptunium nitrate and lanthanum nitrate at a potential of approximately fifty volts and a current density of between about 1.8 and 4.7 milliamperes per square decimeter.

**References Cited in the file of this patent**

**UNITED STATES PATENTS**

40 902,755 Meyer ----- Nov. 3, 1908  
45 1,115,513 Dennis ----- Nov. 3, 1914

**OTHER REFERENCES**

50 Uranium and Atomic Power by Jack DeMent and H. C. Dake, published by Chemical Publishing Co., Brooklyn, New York, 1941, pages 72, 123, 124, 184.

55 The Heavy Elements, Chem. Eng. News, 24, pages 1193-1198, May 10, 1946.

Plutonium and Other Transuranium Elements, Chem. Eng. News, 25, pages 358-60, 397, Feb. 10, 1947.